

## UNITED STATES PATENT OFFICE

2,500,244

## POLYMERIZATION OF ALPHA OLEFINS

Harry G. Doherty, Woodbury, N. J., assignor to  
Socony-Vacuum Oil Company, Incorporated, a  
corporation of New York

No Drawing. Application April 21, 1949,  
Serial No. 88,895

10 Claims. (Cl. 260—683.1)

**1**  
This invention has to do with the production of synthetic lubricants and, more particularly, has to do with the production of these lubricants by a thermal, non-catalytic treatment of certain types of normally liquid olefins at high temperatures.

In a copending application, Serial No. 761,716, filed on July 17, 1947, abandoned in favor of application Serial No. 104,932, filed July 15, 1949, a process has been described for the preparation of synthetic lubricants of excellent character, namely, high viscosity index, relatively low pour point and satisfactory stability. The process there described involves a thermal, non-catalytic conversion of normal, alpha mono-olefins having between about six and about twelve carbon atoms per molecule. Temperatures of operation range from about 500° F. to about 750° F., preferably from about 600° F. to about 700° F.

Although good yields of these desirable synthetic lubricants are obtained by so treating the aforesaid olefins at temperatures lower than about 700° F., the residence or reaction times required to produce commercially feasible yields is excessively long. As disclosed in the aforesaid copending application, however, yields of synthetic lubricants and the viscosity indices thereof diminish substantially as the temperature is raised above 700° F. and secondary reactions are initiated. Secondary reactions which are considered to be involved at the higher temperatures are:

(1) Degradation or cracking begins, as evidenced by decrease in oil yields;

(2) Cyclization begins, as evidenced by a decline in viscosity index with accompanying increase in gravity and refractive index; and

(3) Volatile non-oily components of the reaction mixtures become progressively more saturated, as indicated by a decrease in bromine addition number and, therefore, less suitable for recycling for further conversion.

As a substantial improvement over the aforesaid process, it has now been discovered that synthetic lubricants possessing the combination of desirable properties referred to above, can be produced at temperatures greater than about 700° F. in good yields and in relatively short time periods. The present process comprises treatment of a normal, alpha mono-olefin having be-

**2**  
tween about six and about fourteen carbon atoms per molecule, in the absence of a catalytic material and in the presence of a minor and effective proportion of a cyclic hydrocarbon, at temperatures greater than about 700° F. and not substantially above about 900° F. for relatively short reaction or residence times.

*Normal, alpha mono-olefins*

10 As indicated above, the mono-olefins of this invention are normal or straight chain alpha mono-olefins and contain between about six and about fourteen carbon atoms per molecule. Such mono-olefins are normally liquid at temperatures 15 of the order of 20-25° C. Illustrative of such mono-olefins are the following: hexene-1, octene-1, decene-1, dodecene-1, tetradecene-1, and the like. Preferred, however, are those having from eight to twelve carbon atoms, with 20 decene-1 representing a particularly desirable olefin. It will be clear from the foregoing examples that an alpha olefin may also be referred to as a 1-olefin.

Not only may the mono-olefins of the aforesaid character be used individually in this invention, but they may also be used in admixture with each other. In addition, olefin mixtures containing a substantial proportion of such mono-olefins may be used. Preferred of such mixtures 30 are those containing a major proportion of a 1-olefin or of 1-olefins. Representative of such mixtures are those obtained by the cracking of paraffin waxes and other paraffin products; those obtained from the Fischer-Tropsch and related processes.

These hydrocarbon mixtures may contain, in addition to the 1-olefin or 1-olefins, such materials as: other olefins, paraffins, naphthenes and aromatics.

40 In many instances, in commercial operation, it will be found desirable to use technical grades of 1-olefins. Mixed olefinic materials derived from thermal cracking of hydrocarbon wax or from the Fischer-Tropsch process constitute satisfactory charging stocks. In this connection, it must be noted that it is suspected that substantially straight chain 1-olefins, that is, 1-olefins in which the length of the side chain (or chains) is short relative to the length of the main chain, and in 45 which the side chain (or chains) is not adjacent

to the terminal double bond, are also suitable, although less advantageous charge stocks for the purpose of the present invention. In view of the unavailability of such olefins, however, no test data can be adduced to confirm this suspicion.

#### Cyclic hydrocarbons

The cyclic materials used herein to inhibit or retard secondary reactions may be aromatic, naphthenic or other carbocyclic hydrocarbons. Typical of such hydrocarbons are benzene, toluene, xylenes, propyl benzenes, octyl benzenes, etc.; naphthalene, 1-methyl naphthalene, 2-methyl naphthalene, polymethyl naphthalenes and naphthalenes having longer alkyl chains; cyclopentane, methyl cyclopentane and the like; cyclohexane, methyl cyclohexane, dimethyl cyclohexane, ethyl cyclohexane, and the like; tetralin, and the like. Hydrocarbon mixtures rich in such cyclic materials may also be used, in place of the individual hydrocarbons. Representative of such mixtures are coal tar fractions, straight run and cracked (non-catalytically and catalytically) petroleum products, completely or partially hydrogenated aromatics and the like.

The structural character of the cyclic hydrocarbons appears to have a considerable influence upon inhibitive efficiency. As discussed in detail hereinbelow and as illustrated by several typical examples, the unsubstituted aromatic hydrocarbons and those substituted with one or more alkyl substituents of short, straight-chain structure are generally much more effective than those substituted with relatively long and/or branched-chain alkyl groups. With a cyclic nucleus substituted with more than one alkyl group, it is preferred that each group be limited to not more than two carbon atoms. In the same connection, the position of a substituent group upon the cyclic nucleus is influential, as demonstrated by the appreciably greater efficacy of 2-methyl naphthalene in contrast to 1-methyl naphthalene.

With regard to the concentration of the cyclic inhibitor or retardant, minor amounts as low as about 0.1 per cent to 20 per cent or more may be used. Preferably, however, minor amounts of the order of about one to about five per cent of the total charge are most effective. As shown in the illustrative examples hereinafter, the effectiveness of the various cyclic materials varies to some extent. For example, three per cent of benzene is excellent; whereas, five per cent or more of toluene is required to obtain a similar degree of improvement and three per cent of toluene provides considerably less improvement. The proper concentration will depend largely on inhibitor selected and conditions used.

#### Reaction conditions

The relatively high temperatures and relatively short reaction times of operation used in the present process, vary inversely with each other. When temperatures of the order of about 700-750° F. are used, reaction times are preferably from about three to about one hour; whereas with temperatures of about 800° F., about one to about one-half hour reaction time is satisfactory. Operation at about 850° F. is attended by reaction times of one-half to one-quarter hour.

The operating temperatures and reaction times are critical features herein, as are the concentration and structure of the cyclic inhibitor previously discussed. As a further note relative to inhibitor structure, with temperatures of about

850° F., it has been found that an unsubstituted cyclic compound or one containing only one normal, short-chain alkyl group is more efficacious. This is particularly illustrated by benzene, cyclohexane and their alkylated derivatives.

The foregoing operating conditions appear to be of importance in the present process, other conditions having less influence. Pressure, for example, does not appear to be critical. It may range from about 100 to about 4,000 pounds per square inch, or even higher.

As indicated above, the present process is a thermal, non-catalytic process related to that described in said copending application Serial No. 761,716. The process is described as non-catalytic inasmuch as polymerization or condensation catalysts are not used. For example, Friedel-Crafts type catalysts such as aluminum chloride have hitherto been used to polymerize olefins, under conditions differing considerably from those recited above. It is with this in mind that the present process is described as "non-catalytic."

#### Examples

In order to illustrate the principles of this invention, the results of a series of typical, and non-limiting, conversions are set forth in tabular form in the several tables shown below. These conversions were carried out in rocking-type bombs (American Instrument Co.). The olefins and cyclic inhibitors were charged to the bombs. The bomb heads were secured and the bombs were flushed with nitrogen to displace air present therein. The bombs were then heated (while rocked) to the desired temperature for the desired length of time. Thereafter, the bombs were either cooled and discharged, or discharged immediately through a condensing system while the reactants were still at the reaction temperature.

It should be noted that the reaction times, recited as "Time, Hours" in the tables, represent the time intervals during which the bombs were maintained at the desired temperature, and do not include the time intervals necessary to heat the bombs and their contents to the desired temperature, and do not include the time intervals necessary to cool the bombs after heat to the bombs has been discontinued. In general, about one and one-half hours are required to raise the temperature from 60-80° F., to 750° F., and about eight hours to cool thereafter to 60-80° F., in runs such as shown in the tables. However, since it has been shown in said application Serial No. 761,716 that substantially no polymerization occurs below 500° F., these times are of little significance. The examples given in the tables were made under directly comparable conditions. The condensation products discharged from the bombs were vacuum topped to remove any unreacted hydrocarbon material and any relatively low boiling products, and then were filtered, as in the runs shown in the tables. To distinguish the condensation products from the distillate fractions thereof, the refined oils are identified as "residual oils." The latter term identifies the oils from which unreacted materials and products of intermediate boiling range have been separated.

All of the tests and analyses to which the residual oils in the tables were subjected are well known standard tests. In this connection, it will be noted that the designation "N. N." refers to the neutralization number, which is a measure of the acidity of the oil.

In Table I below, several comparable runs are shown for conversions of decene-1 with and without cyclic inhibitors.

is used. While benzene is greatly superior to toluene when used in three per cent concentration, the two cyclic compounds are of the same

TABLE I

| Run No.                            | 1                            | 2                | 3                  | 4                  | 5                  | 6                     | 7                     | 8                  | 9                   |
|------------------------------------|------------------------------|------------------|--------------------|--------------------|--------------------|-----------------------|-----------------------|--------------------|---------------------|
| Olefin                             | Decene-1                     | Decene-1         | Decene-1           | Decene-1           | Decene-1           | Decene-1              | Decene-1              | Decene-1           | Decene-1            |
| Parts by Weight                    | 740.                         | 400.             | 388.               | 390.               | 388.               | 388.                  | 380.                  | 388.               | 388.                |
| Cyclic Inhibitor                   | None                         | None             | Benzene            | Benzene            | Toluene            | Toluene               | Toluene               | Xylene             | Ethyl benzene       |
| Parts by Weight                    |                              |                  | 12.                | 20.                | 12.                | 12.                   | 20.                   | 12.                | 12.                 |
| Wt. Percent Total Charge           |                              |                  | 3.                 | 5.                 | 3.                 | 3.                    | 5.                    | 3.                 | 3.                  |
| Temperature, °F.                   | 750.                         | 750.             | 750.               | 750.               | 750.               | 750.                  | 750.                  | 750.               | 750.                |
| Reaction Time, Hrs.                | 3.                           | 3.               | 3.                 | 3.                 | 3.                 | 3.                    | 3.                    | 3.                 | 3.                  |
| Max. Pressure, p. s. i. g.         | 600.                         | 700.             | 400.               | 750.               | 1000.              | 2000.                 | 500.                  | 650.               | 500.                |
| Residual Oil:                      |                              |                  |                    |                    |                    |                       |                       |                    |                     |
| Yield, Wt. Percent Olefin Charged. | 30.0.                        | 32.8.            | 46.6.              | 39.8.              | 21.1.              | 23.7.                 | 43.3.                 | 42.8.              | 47.9.               |
| V. I.                              | 116.4                        | 120.4.           | 134.3.             | 128.7.             | 123.4.             | 116.2.                | 127.9.                | 139.1.             | 135.5.              |
| Viscosity @ 100° F., Cs.           | 2 <sup>1</sup> .86           | 21.16            | 24.77              | 18.84              | 25.89              | 30.93                 | 18.25                 | 21.71              | 32.46               |
| Viscosity @ 210° F., Cs.           | 4.29                         | 4.24             | 4.87               | 4.01               | 5.21               | 5.32                  | 3.93                  | 4.51               | 5.94                |
| Pour Point, °F.                    | +10                          | +15              | +15                | +10                | +10                | +20                   | +20                   | +5                 |                     |
| Specific Gravity                   | 0.8639                       | 0.8581           | 0.8453             | 0.8478             |                    |                       | 0.8509                | 0.823              |                     |
| N. N.                              | 1.5                          | Nil              | 0.3                |                    |                    |                       | 0.1                   | Nil                |                     |
| Color (Lovibond)                   | 100.                         | 12.              | 9.                 |                    |                    |                       | 30.                   | 1.5.               | <0.1.               |
| Carbon Residue (Ramsbottom)        | 0.06                         | 0.02             | 0.03               |                    |                    |                       | 0.05                  | 0.03               |                     |
| Run No.                            | 10                           | 11               | 12                 | 13                 | 14                 | 15                    | 16                    |                    |                     |
| Olefin                             | Decene-1                     | Decene-1         | Decene-1           | Decene-1           | Decene-1           | Decene-1              | Decene-1              | Decene-1           | Decene-1            |
| Parts by Weight                    | 388.                         | 388.             | 388.               | 388.               | 388.               | 388.                  | 388.                  | 388.               | 388.                |
| Cyclic Inhibitor                   | Isopropyl benzene.           | t-butyl benzene. | Sec. Amyl benzene. | Sec. Amyl benzene. | Naphthalene.       | 2-methyl naphthalene. | 1-methyl naphthalene. |                    |                     |
| Parts by Weight                    | 12.                          | 12.              | 12.                | 12.                | 12.                | 12.                   | 12.                   | 12.                | 12.                 |
| Wt. Percent Total Charge           | 3.                           | 3.               | 3.                 | 3.                 | 3.                 | 3.                    | 3.                    | 3.                 | 3.                  |
| Temperature, °F.                   | 750.                         | 750.             | 750.               | 750.               | 750.               | 750.                  | 750.                  | 750.               | 750.                |
| Reaction Time, Hrs.                | 3.                           | 3.               | 3.                 | 3.                 | 3.                 | 3.                    | 3.                    | 3.                 | 3.                  |
| Max. Pressure, p. s. i. g.         | 550.                         | 600.             | 525.               | 656.               | 500.               | 900.                  | 900.                  | 1500.              |                     |
| Residual Oil:                      |                              |                  |                    |                    |                    |                       |                       |                    |                     |
| Yield, Wt. Percent Olefin Charged. | 29.4.                        | 25.5.            | 30.2.              | 26.0.              | 24.7.              | 35.8.                 | 24.7.                 |                    |                     |
| V. I.                              | 123.4                        | 121.8.           | 120.2.             | 121.9.             | 121.6.             | 137.5.                | 114.6.                |                    |                     |
| Viscosity @ 100° F., Cs.           | 30.07                        | 29.03            | 28.03              | 35.12              | 40.63              | 22.35                 | 31.44                 |                    |                     |
| Viscosity @ 210° F., Cs.           | 5.35                         | 5.20             | 5.06               | 5.91               | 6.55               | 4.58                  | 5.35                  |                    |                     |
| Pour Point, °F.                    | +30                          |                  |                    |                    |                    |                       |                       |                    |                     |
| Specific Gravity                   |                              |                  |                    |                    |                    |                       |                       |                    |                     |
| N. N.                              |                              |                  |                    |                    |                    |                       |                       |                    |                     |
| Color (Lovibond)                   | 14.                          | 32.              | 18.                | 50.                | 18.                |                       |                       |                    |                     |
| Carbon Residue (Ramsbottom).       |                              |                  |                    |                    |                    |                       |                       |                    |                     |
| Run No.                            | 17                           | 18               | 19                 | 20                 | 21                 | 22                    | 23                    |                    |                     |
| Olefin                             | Decene-1                     | Decene-1         | Decene-1           | Decene-1           | Decene-1           | Decene-1              | Decene-1              | Decene-1           | Decene-1            |
| Parts by Weight                    | 388.                         | 388.             | 380.               | 380.               | 380.               | 380.                  | 380.                  | 380.               | 380.                |
| Cyclic Inhibitor                   | Aromatic Stock. <sup>1</sup> | Cyclohexane      | Cyclohexane        | Methyl Cyclohexane | Methyl Cyclohexane | Ethyl Cyclohexane     | Methyl Cyclopentane   | Ethyl Cyclopentane | Methyl Cyclopentane |
| Parts by Weight                    | 12.                          | 12.              | 20.                | 20.                | 20.                | 12.                   | 20.                   | 12.                | 20.                 |
| Wt. Percent Total Charge           | 3.                           | 3.               | 5.                 | 5.                 | 5.                 | 3.                    | 5.                    | 3.                 | 5.                  |
| Temperature, °F.                   | 750.                         | 750.             | 750.               | 750.               | 750.               | 750.                  | 750.                  | 750.               | 750.                |
| Reaction Time, Hrs.                | 3.                           | 3.               | 3.                 | 3.                 | 3.                 | 3.                    | 3.                    | 3.                 | 3.                  |
| Max. Pressure, p. s. i. g.         | 1200.                        | 525.             | 400.               | 675.               | 475.               | 300.                  | 800.                  |                    |                     |
| Residual Oil:                      |                              |                  |                    |                    |                    |                       |                       |                    |                     |
| Yield, Wt. Percent Olefin Charged. | 34.8.                        | 40.5.            | 41.0.              | 51.7.              | 42.7.              | 42.0.                 | 43.5.                 |                    |                     |
| V. I.                              | 123.1                        | 129.3.           | 134.               | 133.7.             | 126.8.             | 135.4.                | 128.3.                |                    |                     |
| Viscosity @ 100° F., Cs.           | 35.59                        | 28.90            | 21.35              | 17.44              | 22.79              | 23.64                 | 20.05                 |                    |                     |
| Viscosity @ 210° F., Cs.           | 6.00                         | 5.33             | 4.40               | 3.87               | 4.51               | 4.72                  | 4.17                  |                    |                     |
| Pour Point, °F.                    | +15                          | +10              | +15                | +10                | +10                | +5                    | +20.                  |                    |                     |
| Specific Gravity                   | 0.8545                       | 0.8458           | 0.8423             | 0.8478             | 0.8443             | 0.8493                | 0.8493                |                    |                     |
| N. N.                              | 0.2                          | 0.1              | 0.1                | 0.1                | 0.2                | 0.1                   | 0.1                   |                    |                     |
| Color (Lovibond)                   | 46.                          | 5.               | 3.6.               | 8.                 | 4.                 | 17.                   |                       |                    |                     |
| Carbon Residue (Ramsbottom).       | Nil                          | 0.01             | 0.01               | 0.02               | 0.02               | 0.02                  | 0.05                  |                    |                     |

<sup>1</sup> Aromatic Stock is a refinery cut of the following approximate composition: 88% dimethylnaphthalene; 6.5% fluorene; 2.5% phenanthrene. It may contain some trimethylnaphthalenes.

The results shown above in Table I demonstrate the varying degrees of improvement realized with certain cyclic inhibitors. For example, runs 1-4 reveal the substantial improvement in yield and V. I. obtained with benzene incorporated in the decene-1 charge. Runs 5-7 were made with toluene as the inhibitor, and indicate that three per cent of toluene is insufficient to bring about improvement. Yield and V. I. are enhanced, however, when five per cent of toluene

order of effectiveness in five per cent concentration.

Xylene and ethyl benzene are effective in three per cent concentration, as shown by runs 8 and 9.

Runs 1013 reveal that three per cent is an insufficient concentration when benzene carries as a substituent an alkyl group of three or more carbon atoms.

Run 14 reveals that three per cent is an insufficient quantity when naphthalene is the cyclic

material. In contrast, Run 15 indicates that 2-methyl naphthalene is excellent as an inhibitor when used in three per cent concentration. Surprisingly, 1-methyl naphthalene is ineffective in three per cent concentration, as shown by Run 16. Dimethyl naphthalenes are shown to be effective in Run 17.

Runs 18-22 reveal the substantial improvement in yield and V. I. obtained with naphthalene inhibitors. Runs 19-21 demonstrate that yield and V. I. are further enhanced when methyl cyclohexane is used in five per cent concentration.

Considering the results in Table I further, it will be noted that, in three to five per cent concentration, the most effective aromatic inhibitors are benzene, xylenes, ethyl benzene, cyclohexane, methylcyclohexane, dimethylcyclohexane, and ethylcyclohexane, 2-methyl naphthalene and dimethyl naphthalenes.

The series of runs set forth in Table II serve to indicate the influence of higher temperature upon the conversion of decene-1 and upon the activity of cyclic inhibitors.

generally characterized by phosphorus, sulfur, nitrogen, etc., content; representative of such materials is a phosphorus- and sulfur-containing reaction product of pinene and  $P_2S_5$ . Typical detergents which may be so used are metal salts of alkyl-substituted aromatic sulfonic or carboxylic acids, as illustrated by diwax benzene barium sulfonate and barium phenate, barium carboxylate of a wax-substituted phenol carboxylic acid. Extreme pressure agents are well known; illustrating such materials are numerous chlorine and/or sulfur containing compositions, one such material being a chlornaphtha xanthate. Silicones, such as dimethyl silicone, may be used to illustrate foam suppressing compositions. Viscosity index improving agents which may be used are typified by polypropylenes, polyisobutylenes, polyacrylate esters, and the like.

Contemplated also as within the scope of this invention is a method of lubricating relatively moving surfaces by maintaining therebetween a film consisting of any of the aforesaid oils.

It is to be understood that the foregoing description and representative examples are non-

Table II

| Run No.                            | 1          | 2          | 3        | 4                  | 5                           |
|------------------------------------|------------|------------|----------|--------------------|-----------------------------|
| Olefin                             | Decene-1   | Decene-1   | Decene-1 | Decene-1           | Decene-1                    |
| Parts by Weight                    | 700        | 400        | 388      | 380                | 388                         |
| Cyclic Inhibitor                   | None       | None       | Benzene  | Methyl Cyclohexane | Sec.-Amyl-Benzene           |
| Parts by Weight                    |            |            | 12       | 20                 | 12                          |
| Wt. Per Cent Total Charge          |            |            | 3        | 5                  | 3                           |
| Temperature, °F.                   | 850        | 850        | 850      | 850                | 850                         |
| Reaction Time, Hrs.                | 1/4        | 1/4        | 1/4      | 1/4                | 1/4                         |
| Max. Pressure, p. s. i. g.         | 2500       | 2000       | 750      | 950                | 1800                        |
| Residual Oil:                      |            |            |          |                    |                             |
| Yield, Wt. Per Cent Olefin Charged | 6.3        | 4.7        | 25.2     | 23.7               | 5.0                         |
| V. I. of Polymer Oil               | Below Zero | Below Zero | 140      | 102.5              | Too tarry for determination |
| Viscosity @ 100° F., Cs.           | 1738       | 195.6      | 20.06    | 12.17              |                             |
| Viscosity @ 210° F., Cs.           | 24.87      | 10.86      | 4.29     | 2.94               |                             |
| Pour Point, °F.                    | +45        |            | +20      | -25                |                             |
| Specific Gravity                   |            |            | 0.8413   | 0.8676             |                             |
| N. N.                              | 0.8        |            |          | 0.3                |                             |
| Color (Lovibond)                   |            |            | 3.5      |                    |                             |
| Carbon Residue (Ramsbottom)        |            | 2.7        | 0.07     | 0.5                |                             |

In Table II, Runs 1-3 show the high degree of improvement obtained with benzene. Run 4 shows a similar improvement obtained with methyl cyclohexane. Secondary-amyl benzene is shown to be ineffective in three per cent concentration at 850° F., the result being similar to that obtained at 750° F.

As will be evident from the data presented above in Tables I and II, the condensation products of this invention are highly desirable lubricants per se. They are also of considerable value as blending agents for other lubricating oils. They impart desirable viscosity index (V. I.) and pour point characteristics to the oils in combination therewith, for, as indicated above, they have advantageous viscosity index and pour point properties. In short, the synthetic oils find utility in "upgrading" other lubricants. Typical oils with which the synthetic oils may be blended are mineral oils such as are normally used in internal combustion and turbine engines. When so blended, the synthetic oils may comprise the major proportion of the final blended oil, or may even comprise a minor proportion thereof.

One or more of the individual properties of the synthetic lubricants of this invention may be further improved by incorporating therewith a small, but effective amount, of an addition agent such as an antioxidant, a detergent, an extreme pressure agent, a foam suppressor, a viscosity index (V. I.) improver, etc. Antioxidants which may be used are well known in the art, and are

limiting and serve to illustrate the invention, which is to be broadly construed in the light of the language of the appended claims.

I claim:

1. The method for preparing a viscous oil from a normal, alpha mono-olefin having from about six to about fourteen carbon atoms per molecule, which comprises: thermally and non-catalytically heating a hydrocarbon charge consisting essentially of said olefin in the presence of a minor and effective amount of a cyclic hydrocarbon, at a temperature greater than about 700° F. for a period of time from about one hour to about three hours, and less than about 900° F. for a period of time from about one-half hour to about one-quarter hour.
2. The method for preparing a viscous oil from a normal, alpha mono-olefin having from about six to about fourteen carbon atoms per molecule, which comprises: thermally and non-catalytically heating a hydrocarbon charge consisting essentially of said olefin in the presence of a minor and effective amount of a cyclic hydrocarbon, at a temperature greater than about 750° F. for a period of time from about one hour to about three hours, and less than a temperature of about 850° F. for a period of time from about one-half hour to about one-quarter hour.
3. The method for preparing a viscous oil from a normal, alpha mono-olefin having from about eight to about twelve carbon atoms per molecule, which comprises: thermally and non-catalytically

heating a hydrocarbon charge consisting essentially of said olefin in the presence of a minor and effective amount of a cyclic hydrocarbon, at a temperature greater than about 700° F. for a period of time from about one hour to about three hours, and less than about 900° F. for a period of time from about one-half hour to about one-quarter hour.

4. The method for preparing a viscous oil from n-decene-1, which comprises: thermally and non-catalytically heating a hydrocarbon charge consisting essentially of said olefin in the presence of a minor and effective amount of a cyclic hydrocarbon, at a temperature greater than about 750° F. for a period of time from about one hour to about three hours, and less than a temperature of about 850° F. for a period of time from about one-half hour to about one-quarter hour.

5. The method for preparing a viscous oil from a normal, alpha mono-olefin having from about six to about fourteen carbon atoms per molecule, which comprises: thermally and non-catalytically heating a hydrocarbon charge consisting essentially of said olefin in the presence of a minor and effective amount of a cyclic hydrocarbon selected from the group consisting of benzene, xylenes, ethylbenzene, cyclohexane, methyl cyclohexane, dimethyl cyclohexane, ethyl cyclohexane, 2-methyl naphthalene and dimethyl naphthalenes, at a temperature greater than about 700° F. for a period of time from about one hour to about three hours, and less than about 900° F. for a period of time from about one-half hour to about one-quarter hour.

6. The method for preparing a viscous oil from a normal, alpha mono-olefin having from about six to about fourteen carbon atoms per molecule, which comprises: thermally and non-catalytically heating a hydrocarbon charge consisting essentially of said olefin in the presence of a minor and effective amount of a naphthene, at a temperature greater than about 700° F. for a period of time from about one hour to about three hours, and less than about 900° F. for a period of time from about one-half hour to about one-quarter hour.

7. The method for preparing a viscous oil from

a normal, alpha mono-olefin having from about six to about fourteen carbon atoms per molecule, which comprises: thermally and non-catalytically heating a hydrocarbon charge consisting essentially of said olefin in the presence of a minor and effective amount, from about one per cent to about five per cent, of a cyclic hydrocarbon, at a temperature greater than about 700° F. for a period of time from about one hour to about three hours, and less than about 900° F. for a period of time from about one-half hour to about one-quarter hour.

10 8. The method for preparing a viscous oil from n-decene-1, which comprises: thermally and non-catalytically heating a hydrocarbon charge consisting essentially of n-decene-1 in the presence of about three per cent by weight of methyl cyclohexane, at about 750° F. for about three hours.

15 9. The method for preparing a viscous oil from n-decene-1, which comprises: thermally and non-catalytically heating a hydrocarbon charge consisting essentially of n-decene-1 in the presence of about three per cent by weight of xylene, at about 750° F. for about three hours.

20 10. The method for preparing a viscous oil from n-decene-1, which comprises: thermally and non-catalytically heating a hydrocarbon charge consisting essentially of n-decene-1 in the presence of about three per cent by weight of benzene, at about 850° F. for about one-half hour.

HARRY G. DOHERTY.

#### REFERENCES CITED

The following references are of record in the 35 file of this patent:

#### UNITED STATES PATENTS

| Number    | Name       | Date         |
|-----------|------------|--------------|
| 2,450,451 | Schmerling | Oct. 5, 1948 |

#### 40 OTHER REFERENCES

Tilichayev et al.: Proc. Conference on Cracking (Russ.) pages 261-280 (1931).

Nemtsov et al.: J. Gen'l. Chem. (Russ.), vol. 8, 45 pages 1314-1324 (1938).

Egloff: "Reactions of Pure Hydrocarbons," pages 366-7, Reinhold Pub. Corp., N. Y. (1937).

**Certificate of Correction**

**Patent No. 2,500,244**

**March 14, 1950**

**HARRY G. DOHERTY**

It is hereby certified that error appears in the printed specification of the above numbered patent requiring correction as follows:

Column 6, line 70, for "Runs 1013" read *Runs 10-13*; column 7, line 55, for the word "coils" read *oils*;

and that the said Letters Patent should be read as corrected above, so that the same may conform to the record of the case in the Patent Office.

Signed and sealed this 19th day of December, A. D. 1950.

**[SEAL]**

**THOMAS F. MURPHY,**  
*Assistant Commissioner of Patents.*